

## UNITED STATES PATENT OFFICE

2,257,105

## PREPARATION OF RELIEF PRINTING SHEETS ADAPTED FOR USE IN HECTOGRAPHIC REPRODUCTION OF PHOTOGRAPHS

William J. Champion, La Grange, Ill., assignor to Ditto, Incorporated, Chicago, Ill., a corporation of West Virginia

No Drawing. Application June 30, 1939,  
Serial No. 282,300

11 Claims. (Cl. 101—149)

The invention relates to the multiple reproduction of photographic images by contact transfer methods and includes the preparation of relief printing sheets for use therein.

An object of this invention is the provision of photographic reproductions in the form of a gelatin washed-out relief image on a backing, the gelatin relief image being capable of absorbing and holding water soluble basic hectograph dyes in such quantity and with such sharpness as to make possible commercially satisfactory hectograph duplication of the images.

Another object is the hectograph duplication of half tone images, photographic pictures and like images having graduated tones.

Another object is the provision of means whereby representations in color obtained by photographic methods may be reproduced by a hectograph process.

Other objects and advantages of the invention will become apparent as the following detailed description progresses.

In accordance with this invention, a photographic reproduction is produced on a backing in the form of a washed-out moderately tanned gelatin relief. The relief image (known as a matrix) is saturated with a water soluble basic hectograph dye. The dye matrix so obtained contains surplus dye which in accordance with this invention is removed in a manner selected from the following:

(a) The matrix is washed with a salt solution which is substantially a non-solvent for the basic dye; or

(b) The matrix is subjected to a solution of an alkali which fixes the dye stuff in the form of its free base on the gelatin matrix, and the matrix containing this fixed dye base is washed with a non-solvent for the dye base. Then prior to use of the matrix as a printing sheet or hectograph master the dye base is converted back to the water soluble basic dye.

Suitable relief matrices may be made in several ways. In one method, a bichromated gelatin on a film is exposed to light through the film backing in accordance with an image on a negative. The exposed portions of the gelatin become tanned and the unexposed portions remain untanned. On washing the gelatin with hot water the exposed portions remain as a gelatin relief image. A method of this general type is described in Shepherd and Bartlett Patent No. 728,310. This method, while in general operative, is not preferred since even with careful control of the time of exposure the gelatin is apt

to tan and harden not uniformly and to such extent that satisfactory absorptions of hectograph dyes cannot be obtained, particularly for a reproduction of images having graduated tones. Another method which is more satisfactory is to produce a silver image by exposure through the back of an ordinary emulsion coated film and then cause the emulsion contiguous to the silver image to harden by placing it in a bath containing a tanning developer and a substance which decreases the action of the tanning developer. A suitable tanning modifier or neutralizer for this purpose is sodium sulfite. This method gives fairly satisfactory results but is not preferred for the reproduction of images having graduated tones since the tanning developer reacts to some extent with the gelatin which is not contiguous to the silver image. A more suitable method is to produce the silver image by exposure through the back of an ordinary emulsion coated film, then developing the emulsion with a non-tanning developer and after development causing the emulsion contiguous to the silver image to harden by means of a so-called tanning-bleach solution, which is a solution containing an agent such as bicromate which reacts with the metallic silver of the image to form a reduction product which renders insoluble the gelatin contiguous to the silver image, and which also contains a neutralizing agent for the bichromate such as sulfuric acid. This latter method in general gives satisfactory results.

Where it is desired to obtain a faithful reproduction of images, particularly those having graduated tones ranging from high lights to very dark tones, it is important that the penetration of the printing light through the negative be limited in accordance with the density of the negative. This may be done in various ways, among which may be mentioned the exposure of the sensitized emulsion on the relief film through its transparent support and the limitation of the depth to which the rays of exposure light penetrate by having the actinic rays of the exposure light and the emulsion complementary in color as described in John Patent No. 1,453,258.

A process which has given good results in the reproduction of images having graduated tones and which is also suitable for reproduction of images of printed matter and other representations having strongly contrasting lines is as follows:

A negative is employed to make prints by contact or enlargement on a silver halide gelatin emulsion carried by a transparent support. A

suitable emulsion coated film for this purpose is known to the trade at the time of filing this application as Eastman wash-off relief film. The emulsion of this film is of a type which is sensitive only to blue and blue-violet and contains a yellow dye which limits the penetration of the printing light in accordance with the density of the negative. In printing, the exposure is made through the support of the relief film so that the exposed portion of the emulsion is next to the support, not next to the outer surface, because the unexposed portion will be subsequently washed away. In printing, a small amount of light will pass through a high density portion of a negative (corresponding to a highlight in the original subject) and will penetrate the wash-off relief emulsion only a short distance. A shadow in the subject produces a thin deposit of silver in the negative through which the printing light passes and then penetrates deeply into the emulsion.

The next step is the development of the exposed emulsion to produce a silver image. Development is carried to completion using a non-tanning developer such as, for example, hydroquinone or methyl paraaminophenol. The resulting silver image varies in depth from the support directly in proportion to its density.

The next step is to tan the gelatin which is contiguous to the light affected sensitive content of the emulsion, that is, to the silver. This is done by a so-called tanning-bleach solution which contains a tanning neutralizer. A suitable solution is as follows:

(A) Water c. c. 500  
Ammonium bichromate grams 20  
Sulfuric acid C.P. c. c. 4  
Water to make one liter.

(B) Sodium chloride grams 45  
Water to make one liter.

The films are placed in a bath composed of one part of A, one part of B, and 6 parts of water. Sufficient treatment is given to bleach the silver of the positive to a faint brownish image, the time being of the order of 4 minutes.

By the above treatment the silver of the image is converted to silver chloride and the gelatin is tanned and hardened wherever there is metallic silver but is not tanned and hardened where the silver halide grains were not developed. The gelatin is moderately and uniformly tanned by this treatment. Care is taken that the treatment with the tanning bleach is not carried out to such an extent as to completely tan the gelatin in any portions. The moderately tanned gelatin is insoluble in warm water and varies in thickness in accordance with the density of the image.

The next step is the production of the relief image or matrix. This may be done by placing the film in a tank of water at 52° C. The films are lifted completely from the water and replaced about every ten seconds in order that the melted emulsion may drain from the films. By this means the soluble gelatin is removed and a relief image of moderately tanned gelatin obtained which varies in thickness in accordance with the density of the image.

The next treatment after the production of the gelatin relief image by washing with warm water is the removal of the remaining silver chloride from the gelatin. This step is preferred although it is not an essential step. The silver chloride is removed by soaking the relief film

in a fixing solution which will not bring about further tanning of the gelatin. Such a fixing solution is a pure aqueous solution of sodium thiosulphate.

It is apparent that the procedure up to this point is similar to the procedure of the Eastman wash-off relief process described in the publication of Eastman Kodak Company entitled "Color Printing with Eastman Wash-Off Relief Film," No. 7734-2-39, the main differences being that greater care is taken to produce a moderately tanned gelatin than is necessary or called for in the Eastman process.

The next step in the preferred process of this invention is to soak the matrix in a solution of a water soluble basic dye. The amount of dye taken up by the matrix is proportional to the height of the relief image. The moderately tanned gelatin relief image obtained as above will absorb substantial quantities of water soluble basic dyes used in hectograph duplication such as, for example, the water soluble basic triphenyl methane dyes and the water soluble basic xanthene dyes. Such dyes include magenta, methyl violet, malachite green, brilliant green, setacyanide, rhodamines, etc.

After the gelatin matrix has become saturated with a water soluble basic dye (which usually takes five to ten minutes), the film is plunged into a one percent ammonium hydroxide solution. This treatment fixes the dye as a free base onto the gelatin matrix. The free dye base is insoluble in water, and thus while the dye is in the form of the free base the film may be rinsed in running water to remove excess dye without removing any substantial amount of absorbed dye.

After excess dye is removed by washing in water or other non-solvent for the dye base, the dye base is converted back into the water soluble basic dye. When volatile alkalis such as ammonia, morpholine, or the like are used to produce the dye base, the conversion is accomplished by evaporating the volatile alkali. Such evaporation will take place of itself in a short period of time.

The dye containing relief image may be used in its moist or dry condition as a hectograph master. For this purpose the matrix is pressed against a hectograph blanket, thereby transferring portions of the dye to the blanket so that on removal of the matrix a mirror-reverse image will be found on the hectograph blanket. Copies are produced from the hectograph blanket by simply pressing copy sheets against the blanket as is customary in hectograph duplication.

The hectograph master of this invention may be used several times until the dye is exhausted. It then may be re-dyed either with the same or with a different hectograph dye. Thus each master may be used a very great number of times.

The above process is particularly suitable for making reproductions of images having graduated tones. It also, of course, may be used to reproduce printed matter or other representations having strongly contrasting lines.

The process may also be used for reproducing images in color by using, for example, three color record negatives instead of a single monochrome negative. Each color negative is used to produce a separate relief matrix. The relief image obtained from the red-filter negative is dyed with a water soluble basic dye such as

Victoria blue. The print from the green filter negative is dyed with a red water soluble basic dye such as fuchsine. The print from the blue filter negative is dyed with a yellow water soluble basic dye such as auramine.

It is apparent that the process can be varied considerably without departing from the spirit and scope of this invention. There may be used other photographic chemicals producing substantially the same effects or performing substantially the same function as those mentioned above by way of illustration. I may prefer in some instances to apply a slight amount of tanning with a hypo solution, although this tanning should be insufficient to render the gelatin unsuitable to absorb hectograph dyes. Also I may use other alkalis than volatile alkalis to fix the dye as a free base on to the gelatin matrix. However, with the volatile alkalis, conversion of the dye base back to the water soluble basic dye is easily accomplished by simple evaporation of the volatile alkali, whereas when non-volatile alkalis such as sodium hydroxide are used to convert the basic dye to its base the re-conversion must be accomplished by less practical means as for example, the treatment of the dye base with a dilute acid. Furthermore, instead of converting the basic dye stuff into its free base and then washing with water or other non-solvent for the free base to remove excess dye, followed by re-conversion of the free base into the water soluble basic dye stuff, I may use an alternative procedure consisting simply in washing the freshly dyed matrix containing surplus dye with a non-solvent for the water-soluble basic dye stuff employed. For example, I may wash the matrix with a concentrated solution of calcium chloride.

Summing up, it may be stated that the principal advantages of this invention are mainly brought about by the following features:

(1) The gelatin which forms the relief image is prevented from becoming so completely tanned and hardened that it is incapable of absorbing substantial quantities of water soluble basic dye stuffs. Preferably the gelatin of the relief image is produced and then maintained in a moderately tanned condition. For this purpose the use of tanning neutralizer such as disclosed in John Patent No. 1,484,029 is helpful.

(2) Excess dye is removed from the freshly dyed matrix without removing any substantial quantity of absorbed water soluble basic dye. This may be accomplished by either the non-solvent wash method, or by the conversion and re-conversion method described above.

(3) The penetration of the printing light is limited in accordance with the density of the negative so that the actual thickness of the gelatin relief varies in accordance with the density of the image. This feature is particularly important when it is desired to obtain hectograph duplication of half tone images and photographic pictures. It may be accomplished by means such as disclosed in John Patent No. 1,453,258.

While there have been shown and described certain embodiments of the invention, it is to be understood that it is capable of many modifications. Changes, therefore, may be made without departing from the spirit and scope of the invention as described in the appended claims, in which it is the intention to claim all novelty inherent in the invention as broadly as possible, in view of the prior art.

I claim:

1. The method of forming relief printing sheets for use in water color duplicating process which comprises selectively exposing a light sensitized silver halide gelatin emulsion on a transparent support in accordance with an original representation, developing the exposed emulsion to produce a silver image which varies in depth from the support directly in proportion to its density, tanning the gelatin contiguous to the silver image but not to the extent that the gelatin is incapable of further tanning, washing out the unexposed untanned portions of the gelatin to form a matrix having a relief image formed of partially tanned gelatin, applying a water soluble basic dye to the relief image of said matrix, and removing excess dye stuff from said matrix by washing with a concentrated neutral salt solution.
2. The method of forming relief printing sheets for use in water color duplicating process which comprises selectively exposing a light sensitized silver halide gelatin emulsion on a transparent support in accordance with an original representation, developing the exposed emulsion to produce a silver image which varies in depth from the support directly in proportion to its density, tanning the gelatin contiguous to the silver image but not to the extent that the gelatin is incapable of further tanning, washing out the unexposed untanned portions of the gelatin to form a matrix carrying a relief image formed of partially tanned gelatin, applying a water soluble basic dye to the relief image of said matrix, and subjecting the dye containing relief image to a volatile alkali to fix the dye as a free base on to the gelatin matrix, and washing the matrix with a non-solvent for the dye base to remove excess dye prior to the conversion of the dye base back to soluble dye stuff on evaporation of the volatile alkali.
3. The method of forming relief printing sheets for use in water color duplicating process which comprises selectively exposing a light sensitized silver halide gelatin emulsion on a transparent support in accordance with an original representation, developing the exposed emulsion to produce a silver image which varies in depth from the support directly in proportion to its density, tanning the gelatin contiguous to the silver image but not to the extent that the gelatin is incapable of further tanning, washing out the unexposed untanned portions of the gelatin to form a matrix carrying a relief image formed of partially tanned gelatin, applying a water soluble basic dye to the relief image of said matrix, and applying to the dye containing relief image ammonium hydroxide to fix the dye as a free base on to the gelatin matrix, and washing the matrix with water prior to complete evaporation of the ammonia to remove excess dye.
4. The method of forming relief printing sheets for use in water color duplicating processes which comprises forming a matrix carrying a washed-out relief image by selectively exposing a light sensitized silver halide gelatin layer on a transparent support in accordance with an original representation, developing the light sensitized portion with a developer which has substantially no tanning action on the unexposed portions, applying to the matrix a tanning agent and a tanning neutralizer to moderately tan the gelatin contiguous to the light affected sensitive content, washing out the unexposed untanned portion of the matrix to ob-

tain a relief image, dissolving the silver halide from the matrix without tanning the gelatin by applying a fixing agent to the matrix in the absence of a tanning agent in sufficient quantity to substantially further tan the gelatin, applying a water soluble basic dye to the incompletely tanned relief image, subjecting the dye containing image to a solution of a volatile alkali, and washing the image with a non-solvent for the dye base.

5. The method of forming relief printing sheets for use in water color duplicating processes which comprises forming a matrix carrying a washed out relief image by selectively exposing a light sensitized silver halide gelatin layer on a transparent support in accordance with an original representation, developing the light sensitized portion with a developer which has substantially no tanning action on the unexposed portions, applying to the matrix bichromate and sulfuric acid to moderately tan the gelatin contiguous to the light affected sensitive content, washing out the unexposed untanned portion of the matrix to obtain a relief image, dissolving the silver halide from the matrix without tanning the gelatin by applying a fixing agent to the matrix in the absence of a tanning agent in sufficient quantity to substantially further tan the gelatin, applying a water soluble basic dye to the incompletely tanned relief image, subjecting the dye containing image to a dilute ammonium hydroxide, and washing the image with water to remove excess dye.

6. The process of forming relief printing sheets for use in water color duplicating processes which comprises selectively exposing a light sensitized silver halide gelatin emulsion on a transparent support in accordance with an original representation, developing the exposed emulsion to produce a silver image which varies in depth from the support directly in proportion to its density, tanning gelatin contiguous to the silver image but not to the extent that the gelatin is incapable of further tanning, washing out the unexposed untanned portions of the gelatin to form a matrix carrying a relief image, subjecting the matrix to a fixing bath adapted to fix without substantial tanning action on the gelatin, substantially saturating the relief image with a basic dye, and subjecting the dyed image

to a solution of a volatile alkali to fix the dye as a free base on the matrix and allow the removal of excess dye with a minimum of absorbed dye.

5. As an intermediate product in the preparation of relief printing sheets capable of use as a hectograph master; a relief image on a backing, said relief image containing a water insoluble base of a water soluble basic dye stuff.

10 8. As an intermediate product in the preparation of relief printing sheets capable of use as a hectograph master; a photographic reproduction in the form of a gelatin relief, said gelatin relief containing a water insoluble base of a basic dye selected from the group consisting of triphenyl methane and xanthene dye stuffs.

15 9. The method of duplicating which comprises forming a matrix carrying a washed-out relief image by selectively exposing a light sensitized silver halide gelatin emulsion on a transparent support in accordance with an original representation, developing the exposed emulsion to produce a silver image which varies in depth from the support directly in proportion to its density, tanning the gelatin contiguous to the silver but not to the extent that the gelatin is incapable of further tanning, washing out the unexposed, untanned portions of the gelatin to form a matrix having a relief image formed of partially tanned gelatin, applying a water soluble basic dye to the relief image of said matrix, pressing said matrix on a hectograph blanket to transfer the dye image thereto, and making impressions from the dye image on said hectograph blanket.

20 30 35 10. A hectograph master comprising a backing sheet having thereon a moderately tanned gelatin relief image of substantially uniform hardness containing a water soluble basic dye.

11. A hectograph master comprising a backing sheet having thereon a photograph reproduction of an image having graduated tones, said photograph reproduction being in the form of an incompletely tanned gelatin relief of varying thickness, the thickness corresponding to variations in tones of the image, said gelatin relief containing a substantial amount of water soluble basic dye.

WILLIAM J. CHAMPION.